

Nov. 10, 1931.

F. B. ROOT

1,831,323

ORNAMENTED ARTICLE AND PROCESS OF MAKING SAME

Filed Feb. 28, 1929



Inventor

FRANK B. ROOT.

By Frederick S. Duncan

Attorney

## UNITED STATES PATENT OFFICE

FRANK BRIAN ROOT, OF EAST ORANGE, NEW JERSEY, ASSIGNOR TO CHADELOID CHEMICAL COMPANY, OF NEW YORK, N. Y., A CORPORATION OF WEST VIRGINIA

**ORNAMENTED ARTICLE AND PROCESS OF MAKING SAME**

Application filed February 28, 1929. Serial No. 343,330.

This invention relates to ornamental finishes and coatings produced upon articles of manufacture, and to methods of making the same, and more particularly relates to novel effects obtained in that class of finishes known as "wrinkle finish".

The production of such wrinkle finishes or coatings is a marked departure from the prior art directed to finishes and coatings since in that prior art the attempt has always been to avoid any unevenness of surface and to produce as nearly as can be done an uninterrupted but smooth surface coating. This is true in connection with various types of continuous coatings, so that reference to such coatings as "crackle" finishes which involve discontinuous finishes, need not be considered in this connection. The present invention is also concerned with continuous coatings or finishes but in accordance with the present disclosure the finish instead of being smooth presents a continuous but wrinkled finish.

One of the objects of the present invention is the production of special effects in such wrinkle finishes in which the wrinkling is retained but in which the wrinkling is controlled and accentuated at certain points in the coating.

Another object of this invention is the production of the so-called "pine-tree" effect in such coatings.

A further object of this invention is directed to methods of producing such controlled and accentuated wrinkle finishes and the articles carrying such finishes and coatings.

Other and further objects and advantages will appear from the more detailed description given below, it being understood however that this more detailed description is given by way of explanation and illustration only, and not by way of limitation since various changes therein may be made by those

skilled in the art without departing from the scope and spirit of the present disclosure.

In general it may be stated that wrinkle finishes are desirably produced by applying the desired composition to the surface of an article on which the particular effect is to be produced, and then baking or drying the coated article at a temperature at which the wrinkle finish appears. Such finishes have proved very pleasing and attractive. The wrinkling appears to be due to rapid oxidation of the surface of the applied film resulting in the formation of a skin over the less oxidized material on the interior of the coating, the surface film increasing in volume and expanding laterally. The adhesion of the surface coating material for the surface of the article carrying that coating, prevents expansion beyond the confines of that article, so that the expansion of the oxidized film at the surface of the coating results in a wrinkling of the surface film, the less oxidized material on the interior of the coating flowing into the folds.

The general effect in the wrinkle finish coatings is of a substantially level surface exhibiting more or less minute ridges projecting from the surface and running more or less irregularly over that surface. In the application of the present invention to the modification of these wrinkle finishes and coatings, the wrinkling is controlled so that accentuated effects are obtained at various points of the coating, whereby improved ornamental features are procured.

The drawing is illustrative of the modified effects obtained by the present invention. In that drawing there is shown in the single view an enlarged detail of a portion of the surface at close range the wrinkles and spaces between them being enlarged to disclose more particularly the actual contour of the surface, the accentuated wrinkles giving the so-called pine tree effect being shown.

For producing the desired effects, composi-

tions are chosen which under drying or baking conditions give the particular effect herein denominated "wrinkle" finish. An important component of such compositions is a drying oil. The principal drying oils that need be considered in this connection are China wood or tung oil, linseed oil and perilla oil although other drying oils may be used.

10 Among the less common drying oils there may be mentioned chia, Citicica, walnut, poppy-seed, sunflower, candle nut, lumbang, hempseed, fish, etc. The oils which may thus be used in the production of wrinkle finishes 15 are hereinafter generically referred to as "wrinkling oils". While China wood oil gives satisfactory results in wrinkling finishes, the best results are obtained with these drying oils when they have been blown or 20 partially oxidized or preoxidized.

While a varnish or other composition to be used to produce a wrinkle finish must contain a substantial proportion of a wrinkling oil, admixtures of the non-wrinkling oils may be 25 used so long as the amount of the latter is not sufficient to eliminate the wrinkle finish. In such admixtures for the best effects, not less than half of the oil mixture should be a wrinkling oil. It is obvious that similar considerations apply to admixtures of any number of oils whether of the "wrinkling" or "non-wrinkling" types: in all such cases the best effects are obtained in the finish if the amount of wrinkling oil is at least half of 30 the oil content thereof.

The extent of wrinkling in the finish varies according to the amount of resin that is present in the varnish or composition. For each "wrinkling oil" there is a certain range of 40 oil-to-resin ratios within the limits of which the wrinkling takes place to give the best effect. For example, for blown China wood oil the most practicable limits insofar as the appearance of the finish is concerned is from 45 about 6 to 18 gallons of oil to 100 pounds of resin.

Similarly, for untreated China wood oil, it is about 8 to 25 gallons; for blown perilla, 10 to 30; for blown linseed oil, 14 to 35. There 50 is also a lower limit of the oil-to-resin ratio for the production of the more satisfactorily appearing finishes. This ratio varies with the different wrinkling oils. For blown wood oil, about 5 gallons of the oil to 100 lbs. resin produces a varnish giving a more or less well defined effect. With ratios of wood oil below that mentioned, the wrinkle effect falls off while with higher ratios it is more pronounced. This number which may be referred to as "the lowest wrinkling ratio" is 60 a measure of the activity of a wrinkling oil, that is the lower this ratio is, the more powerful is the wrinkling tendency of the oil. 65 The following series expresses the relative

activity of the named wrinkling oils: blown China wood oil 5; China wood oil 6½; blown perilla oil 8; blown linseed oil 12.

7 Of the resins usable in the production of wrinkle finishes and which resins may be denominated "wrinkling finish resins" the following may be noted: Congo, kauri, dammar, Cumar, Pontianak, Manila, Zanzibar, elemi, mastic, phenol-formaldehyde resins particularly of the oil soluble variety, glycerol-phthalic condensation products particularly of the oil soluble variety, paracoumarone, Congo ester, rosin ester, and mixtures of these resins and resin esters.

8 Some substances such as pyroxylin, nitrocellulose, gilsonite, and rosin apparently tend to inhibit the wrinkling effect. Such materials should therefore not be used in proportions to prevent the desired wrinkle finish.

9 In small amounts these substances having a wrinkling inhibiting tendency, produce very fine wrinkles while in large amounts they may completely eliminate wrinkling. Rosin if used in large amount, also tends to produce irregularities in the size and in the 10 interval between wrinkles in the resulting finish.

Solvents or thinners are not a main factor 11 since any moderately volatile solvent can be used. Preferably the major portion of the solvent or thinner should distil below about 325°F. The thinner used may be a mixture of several thinning components. The low boiling thinner evaporates more quickly from the varnish or enamel film, promotes the 12 rapid formation of a surface skin, and during drying assists in maintaining a greater differential between the degree of oxidation of the surface skin and the oil within the film. When the finish is dried at elevated 13 temperatures, the use of low boiling thinners also assists in eliminating any tendency toward sagging of the finish during the drying operation. The following are illustrative of the thinners and solvents that may be used: 14 light naphtha, toluol, benzol, petroleum ether or ligroin (benzine), acetone, carbon tetrachloride, alcohol, chloroform, ethyl acetate, etc., and mixtures of these. To some extent, 15 the character of the finish may be varied by the quantity and character of the thinner used. Turpentine and other high-boiling thinners may also be used. More pronounced wrinkles are produced with compositions containing the lower boiling thinners. 16

Driers and drier combinations are also an important element in the composition since the wrinkled effect appears to be somewhat determined by the rate of oxidation of the wrinkling oil. Such driers as cobalt acetate, red lead, manganese borate, lead linoleate, etc., used alone or in admixture with each other or with the other driers are illustrative.

17 The compositions may be made and applied as either clear varnishes or as pigment-

ed enamels. For example such enamels may be prepared by mixing with the clear varnish compositions, a pigment paste ground in a varnish or a gum solution.

5 To exemplify the types of compositions that may be used in the production of varnishes, etc. that yield wrinkle finishes the following specific examples are noted.

*Example 1*

|    |     |                      |
|----|-----|----------------------|
| 10 | 100 | lbs. cumar           |
|    | 2½  | lbs. lead linoleate  |
|    | ½   | lb. cobalt acetate   |
|    | 7   | gals. blown wood oil |
| 15 | 10  | gals. light naphtha  |
|    | 12  | gals. toluol.        |

*Example 2*

|    |     |                      |
|----|-----|----------------------|
| 20 | 100 | lbs. Congo           |
|    | 4   | lbs. rosin           |
|    | 3½  | lbs. red lead        |
|    | 2   | lbs. manganese oxide |
|    | 10  | gals. wood oil       |
|    | 10  | gals. light naphtha  |
| 25 | 32  | gals. toluol.        |

*Example 3*

|    |     |                         |
|----|-----|-------------------------|
| 30 | 100 | lbs. Congo              |
|    | 5   | lbs. red lead           |
|    | 2½  | lbs. manganese oxide    |
|    | 25  | gals. blown linseed oil |
|    | 10  | gals. light naphtha     |
|    | 18  | gals. toluol.           |

*Example 4*

|    |     |                           |
|----|-----|---------------------------|
| 35 | 100 | lbs. Congo                |
|    | 4   | lbs. rosin                |
|    | 1¾  | lbs. red lead             |
|    | ¾   | lbs. manganese borate     |
|    | 2½  | gals. China wood oil      |
|    | 6½  | gals. blown wood oil      |
| 40 | 4   | gals. blown soya bean oil |
|    | 5   | gals. light naphtha       |
|    | 17  | gals. toluol.             |

Example 1 is exemplary of a varnish that contains blown wood oil as the only wrinkle oil and this composition gives a very uniform effect.

Example 2 illustrates the use of unblown or unoxidized China wood oil. A very good wrinkle effect is obtained with this composition. Blown wood oil and other blown drying oils generally give very desirable and pronounced wrinkle effects, but wood oil untreated is the best of the untreated or un-oxidized drying oils that can be used.

Example 3 illustrates the use of blown linseed oil as the wrinkle oil in the composition. This composition gives a well-defined and a uniform wrinkle effect.

Example 4 illustrates the use of non-wrinkle type of oil specifically given in the example as blown soya bean oil. Raw soya bean oil may be substituted for the blown oil and instead of soya bean oil there may

65 also be used any semi- or non-drying oil such

as cotton seed, corn, castor, rape-seed, rubber-seed, olein, etc.

In producing the improved wrinkle finish of this invention, it is advantageous to dry or bake the applied finish of varnish or enamel, preferably at an elevated temperature depending on the type of article being treated. For metal and related surfaces a temperature of 150° F. up to approximately 450° F. may be advantageously used. For wood and similar materials somewhat lower temperatures such as 120° F. up to 140° F. may be utilized. At elevated temperatures rapid oxidation of the surface of the applied film is promoted and any tendency toward diffusion of oxidation products from the surface into the interior of the film is lessened. In general, drying at elevated temperatures accentuates the wrinkling and assists in providing a harder finish.

As an illustration of drying times and temperatures satisfactory wrangled finishes are obtained with the compositions herein set forth as follows: In five hours at 180° F., in three hours at 200° F., in two hours at 250° F., in one and one-half hours at 300° F., and in three-fourths of an hour at 400° F. Drying at elevated temperatures also assists in making the finish resistant to the action of the usual solvents employed in pyroxylin lacquers and enamels. Increase in the amount of oil in the composition results in wrinkling at lower temperatures and hence when the lower temperatures are to be used in connection with wood and related articles, the compositions may desirably contain more oil. Further the higher oil content gives added flexibility so that the long oil compositions are desirable for use in metal stamping, or on leather, paper, cloth, rubber, etc. Example 4 above, gives a baked film that is quite elastic due to the high oil content.

There have been set forth above a number of considerations directed to the types of compositions and the baking temperatures which effect the character of the wrinkles produced in the finish. Other factors however are also found which affect the character of the wrinkles produced. For example the thickness of the applied film will result in differences in the finish. Thinner films give finer wrinkles and thicker films coarser wrinkles. When spraying is used, spray nozzles giving coarse atomization give greater deposition of composition and consequently coarser wrinkles, while on the other hand spray nozzles of finer atomization give thinner films with finer wrinkles.

In the discussion set forth above the compositions and methods used result in substantially uniformly distributed wrinkle finishes, the character of wrinkle whether coarse or fine being substantially uniform over the surface.

One phase of the present invention is par-

ticularly concerned with the production of such wrinkle finishes in which the texture of the wrinkle is modified at one or more segregated areas in the wrinkled surface so that a 5 design effect is produced in the wrinkle finish. Such modified effects may be referred to for example as sag, curtain and pine-tree. These several effects may be generically referred to as accentuated rugosities or waves of wrinkle 10 finish produced by agglomeration of heavier or thicker films of the composition at certain points of the surface while at other points the regular wrinkle finish serves as a background for the accentuated wrinkled areas. 15 The pine-tree effect is that wherein the accentuated rugosities are more in the nature of inverted V's. The pine-tree effect is well illustrated in the drawing. The areas A, A represent the so-called pine-tree appearance, 20 which when viewed more distantly so that the high lights of the surface are seen, give a distinct pine tree appearance on the more regularly wrinkled background indicated at areas B, B. In order to illustrate the actual 25 contour of the surface, the drawing shows such surface carrying a wrinkled finish enlarged to give greater detail of that surface. The inverted V's at A, A represent the accentuated portions of the surface found on 30 the more regularly wrinkled areas B, B, the latter serving as a background for the accentuated rugosities constituting the pine-tree.

For the production of these wrinkled finishes with accentuated rugosities in the finish 35 the article is desirably coated with a relatively heavy coating of the desired composition and baked in an inclined position which inclined position may vary from a small angle to the horizontal, to a vertical position. The 40 incline of the surface of the article bearing the coating produces a flowing or movement of the wrinkled coating after it is applied and at or about the time when the baking commences and before the baking has caused 45 the setting of the finish to take place to a point where such movement or flowing would be prevented. The effects which are obtained are the resultants of certain forces acting. The inclined or vertical surface is expanding 50 so that there is an outwardly directed force in all directions from the point at which the oil aggregate forms. Gravity also acts to produce a downwardly directed force. The resultants of these forces are vectors 55 acting from the point at which the oil aggregate forms in a direction determined by the two forces referred to above. The angle of the surface of the article being treated may accordingly be varied to regulate the character 60 of these accentuated rugosities, the maximum effect being obtained with the surface in vertical position.

These observations are substantiated by the action of a sprayed panel during the 65 drying or baking operation particularly

under the action of heat. The wrinkling usually starts at the edges and simultaneously there are noted small specks scattered all over the surface which gradually develop into the inverted V's. These areas eventually comprise the pine-trees but the important point is that the wrinkling on the surface of the panel starts at these segregated points, the apices of the V's.

The point at which such wrinkling first appears apparently results from an aggregation of partially polymerized and oxidized molecules. These aggregations may or may not be present as nuclei in the varnish before it is applied but they are helped in their growth by the action of the oven heat and by the vortex current caused by the rapid evaporation of the thinner. The film of compositions should be heavy enough in order to produce pine-trees because in thin films the solvent evaporates quickly and the surface skin forms and wrinkles before the oil aggregates have grown to sufficient size for their influence to be shown. Further it may be stated that of two wrinkling varnishes the one that contains more oil wrinkles in a shorter time than the one with less oil, other factors being equal in the two cases.

The flowing or movement of the wrinkled coating after it is applied which results in the accentuated rugosities at certain points of the coating, may be accomplished in other ways than merely by gravity due to setting the work in a vertical position or at an angle to the horizontal. It may be accomplished for example by air currents or other flowing methods.

Pronounced pine tree effects have also been obtained by the addition to a clear wrinkle varnish of an unground pigment of relatively light gravity. Magnesia suspended in oil may be used for this purpose. The amount of pigment added should be small, say less than 1 per cent based on the total composition and this added pigment should be well distributed in the composition. It is possible that the particles of unground pigment act as an obstruction to the flow of the composition and thus produce the pine tree effect at the point where the pigment becomes fixed in the surface.

When gang sprays are used to apply the composition, at certain points the atomization may be made coarser to produce heavier or thicker layers at these points resulting in coarser wrinkles in such thicker layers. Accentuated rugosities distributed in the more uniformly wrinkled finishes may be produced in this manner.

Accentuated rugosities at certain points of the surface may also be controlled by employing a different temperature at different points during the baking of the sprayed surface. A higher temperature causes a more rapid wrinkling effect than a lower temper-

ature. The effect of localized heating at different points of the surface results in a variation in the type of wrinkle produced at these particular points as compared with 5 the type of wrinkle produced by the action of heat at other places in the surface.

The baked or dried finishes of the present invention are particularly resistant to softening by lacquer compositions and particularly 10 the solvents used in nitrocellulose lacquers.

So that although the rugose surface of the wrinkle finish affords a very extensive area for the action of such solvents or lacquers the baking creates a resistance to such softening 15 action. Consequently the wrinkle finishes and compositions used for producing such coatings are particularly desirable as under-coats where a wrinkle finish is desired and such finishes may then be given one or more 20 coats of pyroxylin enamels, oil enamels, or baking japans. When pigments are used in the wrinkle finish which have a tendency to change or darken under the action of elevated temperatures, these finishes may be coated 25 with pyroxylin lacquer compositions.

While certain theoretical considerations have been set forth above in an attempt to explain some of the effects obtained, it should be understood that this invention is not 30 limited by such theoretical considerations because the compositions and methods discussed above do result in the particular effects set forth and it is immaterial what may be the actual cause of such effects. Pronounced 35 results of the character herein set forth are readily obtained with the compositions and methods outlined above.

Having thus set forth my invention, I claim:

40 1. An ornamented article of manufacture carrying a wrinkle finish coating having accentuated rugosities therein at segregated areas, distributed within the remainder of the wrinkle finish coating.

45 2. An ornamented article of manufacture carrying a wrinkle finish coating having accentuated rugosities formed of films of composition agglomerated at various points therein distributed within the remainder of 50 the wrinkle finish coating.

55 3. An ornamented article of manufacture carrying a wrinkle finish coating having accentuated rugosities of the pine tree type formed of films of composition agglomerated at various points therein into the form of inverted V's, distributed within the remainder of the wrinkle finish coating.

60 4. The process of ornamenting an article of manufacture which comprises applying to the surface thereof a wrinkling finish composition, and drying said coated article under conditions to produce a wrinkle finish coating having accentuated rugosities therein at segregated areas distributed within the remainder of 65 the wrinkle finish coating.

5. The process of ornamenting an article of manufacture which comprises applying to the surface thereof a wrinkling finish composition, and baking said coated article under conditions to produce a wrinkle finish coating having accentuated rugosities therein at segregated areas distributed within the remainder of the wrinkle finish coating. 70

FRANK BRIAN ROOT.

75

80

85

90

95

100

105

110

115

120

125

130